

# United States Patent [19]

Chapman et al.

[11] Patent Number: 5,037,799

[45] Date of Patent: Aug. 6, 1991

[54] YELLOW DYE MIXTURE FOR THERMAL COLOR PROOFING

[75] Inventors: Derek D. Chapman; Steven Evans, both of Rochester, N.Y.

[73] Assignee: Eastman Kodak Company, Rochester, N.Y.

[21] Appl. No.: 628,538

[22] Filed: Dec. 14, 1990

[51] Int. Cl.<sup>5</sup> ..... B41M 5/035; B41M 5/26

[52] U.S. Cl. ..... 503/227; 8/471; 428/195; 428/913; 428/914; 430/200; 430/201; 430/945

[58] Field of Search ..... 8/471; 428/195, 913, 428/914; 430/200, 201, 945; 503/227

## References Cited

### U.S. PATENT DOCUMENTS

4,914,077 4/1990 Shuttleworth et al. ..... 503/227

### OTHER PUBLICATIONS

Chem. Ber., 16, 1082 (1883).

Trans. Faraday Soc., 32, 1318 (1936).

J. Org. Chem., 23, 373 (1958).

Primary Examiner—Bruce H. Hess

Attorney, Agent, or Firm—Harold E. Cole

### ABSTRACT

A yellow dye-donor element for thermal dye transfer comprises a support having thereon a dye layer comprising a mixture of yellow dyes dispersed in a polymeric binder, at least one of the yellow dyes having the formula:



I

wherein:

R¹ represents hydrogen or halogen;

each R² independently represents hydroxy, alkoxy, aryloxy, acyloxy, aminocarbonyl, carbamoyloxy, halogen, aryl, hetaryl, cyano, acylamido, alkoxy carbonyl, alkylthio, arylthio, alkylsulfonyl, arylsulfonyl, alkylsulfonamido or arylsulfonamido; or any

two adjacent R²'s together represent the atoms necessary to complete a 5- or 6-membered fused saturated or aromatic ring;

Y represents H or OH; and

n is an integer from 0 to 4;

or any two adjacent R¹'s together represent the atoms necessary to form a 5- or 6-membered fused ring;

n represents an integer from 0-4; and at least one of the other of the dyes having the formula:



II

wherein:

R³ and R⁴ each independently represents a substituted or unsubstituted alkyl group of from 1 to about 6 carbon atoms, a cycloalkyl group of from about 5 to about 7 carbon atoms; a substituted or unsubstituted allyl group; an aryl group of from about 6 to about 10 carbon atoms; a hetaryl group of from 5 to 10 atoms; acyl; arylsulfonyl; aminocarbonyl; aminosulfonyl; fluorosulfonyl; halogen; nitro; alkylthio; or arylthio;

R⁵ represents H, a substituted or unsubstituted alkyl, allyl, aryl or hetaryl group as described above for R³; halogen; carbamoyl; cyano; or alkoxy carbonyl; each R⁶ independently represents substituted or unsubstituted alkyl, aryl, allyl or hetaryl groups such as those listed above for R³; hydroxy, alkoxy, aryloxy, acyloxy, aminocarbonyl, aminosulfonyl, carbamoyloxy, halogen, aryl, cyano, nitro, trifluoromethyl, fluorosulfonyl, acylamido, alkoxy carbonyl, alkylthio, arylthio, alkylsulfonyl, arylsulfonyl, alkylsulfonamido or arylsulfonamido; or two adjacent R⁶'s together represent the atoms necessary to complete a 5- or 6-membered fused saturated or aromatic ring;

X represents CR⁷ or N;

R⁷ represents the same groups as R⁵; and m is an integer from 0 to 5.

15 Claims, No Drawings

## YELLOW DYE MIXTURE FOR THERMAL COLOR PROOFING

This invention relates to use of a mixture of yellow dyes in a yellow dye-donor element for thermal dye transfer imaging which is used to obtain a color proof that accurately represents the hue of a printed color image obtained from a printing press.

In order to approximate the appearance of continuous-tone (photographic) images via ink-on-paper printing, the commercial printing industry relies on a process known as halftone printing. In halftone printing, color density gradations are produced by printing patterns of dots or areas of varying sizes, but of the same color density, instead of varying the color density continuously as is done in photographic printing.

There is an important commercial need to obtain a color proof image before a printing press run is made. It is desired that the color proof will accurately represent at least the details and color tone scale of the prints obtained on the printing press. In many cases, it is also desirable that the color proof accurately represent the image quality and halftone pattern of the prints obtained on the printing press. In the sequence of operations necessary to produce an ink-printed, full-color picture, a proof is also required to check the accuracy of the color separation data from which the final three or more printing plates or cylinders are made. Traditionally, such color separation proofs have involved silver halide photographic, high-contrast lithographic systems or non-silver halide light-sensitive systems which require many exposure and processing steps before a final, full-color picture is assembled.

Colorants that are used in the printing industry are insoluble pigments. By virtue of their pigment character, the spectrophotometric curves of the printing inks are often unusually sharp on either the bathochromic or hypsochromic side. This can cause problems in color proofing systems in which dyes as opposed to pigments are being used. It is very difficult to match the hue of a given ink using a single dye.

In U.S. patent application 514,643, filed Apr. 25, 1990, of DeBoer, a process is described for producing a direct digital, halftone color proof of an original image on a dye-receiving element. The proof can then be used to represent a printed color image obtained from a printing press. The process described therein comprises:

- a) generating a set of electrical signals which is representative of the shape and color scale of an original image;
- b) contacting a dye-donor element comprising a support having thereon a dye layer and an infrared-absorbing material with a first dye-receiving element comprising a support having thereon a polymeric, dye image-receiving layer;
- c) using the signals to imagewise-heat by means of a diode laser the dye-donor element, thereby transferring a dye image to the first dye-receiving element; and
- d) retransferring the dye image to a second dye image-receiving element which has the same substrate as the printed color image.

In the above process, multiple dye-donors are used to obtain a complete range of colors in the proof. For example, for a full-color proof, four colors: cyan, magenta, yellow and black are normally used.

By using the above process, the image dye is transferred by heating the dye-donor containing the infrared-absorbing material with the diode laser to volatilize the dye, the diode laser beam being modulated by the set of signals which is representative of the shape and color of the original image, so that the dye is heated to cause volatilization only in those areas in which its presence is required on the dye-receiving layer to reconstruct the original image.

Similarly, a thermal transfer proof can be generated by using a thermal head in place of a diode laser as described in U.S. Pat. No. 4,923,846. Commonly available thermal heads are not capable of generating half-tone images of adequate resolution but can produce

high quality continuous tone proof images which are satisfactory in many instances. U.S. Pat. No. 4,923,846 also discloses the choice of mixtures of dyes for use in thermal imaging proofing systems. The dyes are selected on the basis of values for hue error and turbidity.

20 The Graphic Arts Technical Foundation Research Report No. 38, "Color Material" (58-(5) 293-301, 1985 gives an account of this method.

An alternative and more precise method for color measurement and analysis uses the concept of uniform color space known as CIELAB in which a sample is analyzed mathematically in terms of its spectrophotometric curve, the nature of the illuminant under which it is viewed and the color vision of a standard observer. For a discussion of CIELAB and color measurement, see "Principles of Color Technology", 2nd Edition, p.25-110, Wiley-Interscience and "Optical Radiation Measurements", Volume 2, p.33-145, Academic Press.

25 In using CIELAB, colors can be expressed in terms of three parameters:  $L^*$ ,  $a^*$  and  $b^*$ , where  $L^*$  is a lightness function, and  $a^*$  and  $b^*$  define a point in color space. Thus, a plot of  $a^*$  v.  $b^*$  values for a color sample can be used to accurately show where that sample lies in color space, i.e., what its hue is. This allows different samples to be compared for hue if they have similar 30 density and  $L^*$  values.

35 In color proofing in the printing industry, it is important to be able to match the proofing ink references provided by the International Prepress Proofing Association. These ink references are density patches made with standard 4-color process inks and are known as 40 SWOP (Specifications Web Offset Publications) Color References. For additional information on color measurement of inks for web offset proofing, see "Advances in Printing Science and Technology", Proceedings of the 19th International Conference of Printing Research Institutes, Eisenstadt, Austria, June 1987, J. T. Ling and R. Warner, p.55.

45 We have found that an acceptable hue match for a given sample is obtained by a mixture of dyes, if the color coordinates of the sample lie close to the line connecting the coordinates of the individual dyes. Thus, this invention relates to the use of a mixture of yellow dyes for thermal dye transfer imaging to approximate a hue match of the yellow SWOP Color Reference. While the individual dyes by themselves do not match the SWOP Color Reference, the use of a suitable mixture of dyes allows a good color space (i.e., hue) match to be achieved. In addition, the mixture of dyes described in this invention provide a closer hue match to the SWOP standard than the preferred dye of U.S. Patent 4,923,846.

50 Accordingly, this invention relates to a yellow dye-donor element for thermal dye transfer comprising a

support having thereon a dye layer comprising a mixture of yellow dyes dispersed in a polymeric binder, at least one of the dyes having the formula:



wherein:

R<sup>1</sup> represents hydrogen or halogen;  
each R<sup>2</sup> independently represents hydroxy, alkoxy, aryloxy, acyloxy, aminocarbonyl, carbamoyloxy, halogen, aryl, hetaryl, cyano, acylamido, alkoxy carbonyl, alkylthio, arylthio, alkylsulfonyl, arylsulfonyl, alkylsulfonamido or arylsulfonamido; or any two adjacent R<sup>2</sup>'s together represent the atoms necessary to complete a 5- or 6-membered fused saturated or aromatic ring;

Y represents H or OH; and  
n is an integer from 0 to 4;

and at least one of the other of the dyes having the formula:



wherein:

R<sup>3</sup> and R<sup>4</sup> each independently represent an alkyl group of from 1 to about 6 carbon atoms, such as methyl, ethyl, propyl, isopropyl, butyl, pentyl, hexyl; a cycloalkyl group of from about 5 to about 7 carbon atoms such as cyclopentyl, cyclohexyl, etc.; an allyl group; an aryl group of from about 6 to about 10 carbon atoms such as phenyl, naphthyl, etc.; a hetaryl group of from about 5 to about 10 atoms such as thienyl, 50 pyridyl, benzoxazolyl, etc.; or such alkyl, cycloalkyl, allyl, aryl or hetaryl groups substituted with alkyl, aryl, hetaryl, hydroxy, acyloxy, alkoxy, aryloxy, cyano, acylamino, halogen, carbamoyloxy, ureido, imido, alkoxy carbonyl, alkylsulfonyl, arylsulfonyl, nitro, etc.;

R<sup>5</sup> represents H, a substituted or unsubstituted alkyl group of from 1 to about 6 carbon atoms such as those listed above for R<sup>3</sup>; a substituted or unsubstituted allyl, aryl or hetaryl group as described above for R<sup>3</sup>; halogen; carbamoyl; cyano; or alkoxy carbonyl; each R<sup>6</sup> independently represents substituted or unsubstituted alkyl, aryl, allyl or hetaryl groups such as those listed above for R<sup>3</sup>; hydroxy, alkoxy, aryloxy, acyloxy, aminocarbonyl, aminosulfonyl, carbamoyloxy, halogen, aryl, cyano, nitro, trifluoromethyl, fluorosulfonyl, acylamido, alkoxy carbonyl,

alkylthio, arylthio, alkylsulfonyl, arylsulfonyl, alkylsulfonamido or arylsulfonamido; or two adjacent R<sup>6</sup>'s together represent the atoms necessary to complete a 5- or 6-membered fused saturated or aromatic ring;

I 5 X represents CR<sup>7</sup> or N;

R<sup>7</sup> represents the same groups as R<sup>5</sup>; and m is an integer from 0 to 5.

In a preferred embodiment of the invention, R<sup>1</sup>, R<sup>2</sup> and Y in the above structural formula I are each hydrogen.

In another preferred embodiment of the invention, X in the above structural formula II is C—CN. In another preferred embodiment, R<sup>3</sup> is CH<sub>3</sub>OC<sub>2</sub>H<sub>4</sub> or n-C<sub>4</sub>H<sub>9</sub>. In

15 yet still another preferred embodiment, R<sup>4</sup> is CH<sub>3</sub>OC<sub>2</sub>H<sub>4</sub> or n-C<sub>4</sub>H<sub>9</sub>. In still another preferred embodiment, R<sup>5</sup> is CH<sub>3</sub> or C<sub>6</sub>H<sub>5</sub>. In yet still another preferred embodiment, R<sup>6</sup> is CN, OCH<sub>3</sub> or CO<sub>2</sub>C<sub>2</sub>H<sub>5</sub>.

In another preferred embodiment of the invention, in formulas I and II above, R<sup>1</sup>, R<sup>2</sup> and Y are each hydrogen, n is 1, R<sup>3</sup> and R<sup>4</sup> are each CH<sub>3</sub>OC<sub>2</sub>H<sub>4</sub>, R<sup>5</sup> is CH<sub>3</sub>, R<sup>6</sup> is 2,5—(OCH<sub>3</sub>)<sub>2</sub>, X is C—CN and m is 2.

The compounds of formula I above employed in the invention may be prepared by any of the processes disclosed in Chem. Ber., 16, 1082 (1883), Trans. Faraday Soc., 32, 1318 (1936) or J. Org. Chem., 23, 373 (1958), the disclosures of which are hereby incorporated by reference.

The compounds of formula II above employed in the invention may be prepared by any of the processes disclosed in U.S. Pat. No. 4,914,077, the disclosure of which is hereby incorporated by reference.

Compounds included within the scope of formula I above include the following:



| Cmpd | Y  | R <sup>1</sup> | R <sup>2</sup>                                         |
|------|----|----------------|--------------------------------------------------------|
| A    | H  | H              | H                                                      |
| B    | OH | H              | H                                                      |
| C    | OH | H              | 4-CO <sub>2</sub> C <sub>5</sub> H <sub>11</sub>       |
| D    | OH | Br             | 4-CON(C <sub>4</sub> H <sub>9</sub> ) <sub>2</sub>     |
| E    | OH | H              | 4-CO <sub>2</sub> C <sub>8</sub> H <sub>7</sub> -n     |
| F    | OH | Br             | 4-CON(C <sub>3</sub> H <sub>7</sub> ) <sub>2</sub>     |
| G    | H  | H              | 4-CO <sub>2</sub> C <sub>4</sub> H <sub>9</sub> -i     |
| H    | H  | H              | 4,5-Cl <sub>2</sub>                                    |
| I    | OH | Cl             | 3-OC <sub>2</sub> H <sub>5</sub>                       |
| J    | H  | H              | 3-F                                                    |
| K    | H  | H              | 4,5-[CON(CH <sub>3</sub> ) <sub>2</sub> ] <sub>2</sub> |
| L    | OH | H              | 4-C <sub>3</sub> H <sub>7</sub> -i                     |
| M    | H  | H              | 3,6-(OCH <sub>3</sub> ) <sub>2</sub>                   |
| N    | OH | H              | 4-C <sub>6</sub> H <sub>5</sub>                        |
| O    | OH | Br             | 4-NHCOC <sub>2</sub> H <sub>5</sub>                    |
| P    | OH | H              | 3-SO <sub>2</sub> C <sub>4</sub> H <sub>9</sub> -n     |
| Q    | H  | H              | 4,5-(SC <sub>2</sub> H <sub>5</sub> ) <sub>2</sub>     |
| R    | OH | F              | 3-(3-pyridyl)                                          |
| S    | OH | Cl             | 4-(2-thienyl)                                          |
| T    | H  | H              | 3,6-(CN) <sub>2</sub>                                  |

Compounds included within the scope of formula II above include the following:



II

| Cmpd | X    | R <sup>4</sup>                                        | R <sup>3</sup>                                        | R <sup>5</sup>                | R <sup>6</sup>                                                                    |
|------|------|-------------------------------------------------------|-------------------------------------------------------|-------------------------------|-----------------------------------------------------------------------------------|
| 1    | C-CN | CH <sub>3</sub> OC <sub>2</sub> H <sub>4</sub>        | CH <sub>3</sub> OC <sub>2</sub> H <sub>4</sub>        | CH <sub>3</sub>               | 2,5-(OCH <sub>3</sub> ) <sub>2</sub>                                              |
| 2    | C-CN | CH <sub>3</sub> OC <sub>2</sub> H <sub>4</sub>        | CH <sub>3</sub> OC <sub>2</sub> H <sub>4</sub>        | CH <sub>3</sub>               | 4-CO <sub>2</sub> C <sub>2</sub> H <sub>5</sub>                                   |
| 3    | C-CN | n-C <sub>4</sub> H <sub>9</sub>                       | n-C <sub>4</sub> H <sub>9</sub>                       | C <sub>6</sub> H <sub>5</sub> | 2-CN                                                                              |
| 4    | C-CN | CH <sub>3</sub> OC <sub>2</sub> H <sub>4</sub>        | CH <sub>3</sub> OC <sub>2</sub> H <sub>4</sub>        | CH <sub>3</sub>               | 4-Cl                                                                              |
| 5    | C-CN | CH <sub>3</sub> OC <sub>2</sub> H <sub>4</sub>        | CH <sub>3</sub> OC <sub>2</sub> H <sub>4</sub>        | CH <sub>3</sub>               | 3-CO <sub>2</sub> C <sub>2</sub> H <sub>5</sub>                                   |
| 6    | C-CN | n-C <sub>4</sub> H <sub>9</sub>                       | CH <sub>3</sub> OC <sub>2</sub> H <sub>4</sub>        | CH <sub>3</sub>               | 2-OCH <sub>3</sub>                                                                |
| 7    | C-CN | CH <sub>3</sub> OC <sub>2</sub> H <sub>4</sub>        | n-C <sub>4</sub> H <sub>9</sub>                       | CH <sub>3</sub>               | 2-OCH <sub>3</sub>                                                                |
| 8    | C-CN | n-C <sub>4</sub> H <sub>9</sub>                       | n-C <sub>4</sub> H <sub>9</sub>                       | CH <sub>3</sub>               | 2-CF <sub>3</sub>                                                                 |
| 9    | C-CN | n-C <sub>4</sub> H <sub>9</sub>                       | n-C <sub>4</sub> H <sub>9</sub>                       | CH <sub>3</sub>               | 2-CO <sub>2</sub> C <sub>2</sub> H <sub>5</sub>                                   |
| 10   | C-CN | s-C <sub>6</sub> H <sub>11</sub>                      | s-C <sub>6</sub> H <sub>11</sub>                      | CH <sub>3</sub>               | 2-CF <sub>3</sub>                                                                 |
| 11   | C-CN | CH <sub>3</sub> OC <sub>2</sub> H <sub>4</sub>        | CH <sub>3</sub> OC <sub>2</sub> H <sub>4</sub>        | CH <sub>3</sub>               | 2-CO <sub>2</sub> C <sub>2</sub> H <sub>5</sub>                                   |
| 12   | C-CN | n-C <sub>4</sub> H <sub>9</sub>                       | n-C <sub>4</sub> H <sub>9</sub>                       | C <sub>6</sub> H <sub>5</sub> | 2-CF <sub>3</sub>                                                                 |
| 13   | C-CN | n-C <sub>4</sub> H <sub>9</sub>                       | n-C <sub>4</sub> H <sub>9</sub>                       | C <sub>6</sub> H <sub>5</sub> | 2-CO <sub>2</sub> C <sub>2</sub> H <sub>5</sub>                                   |
| 14   | C-CN | CH <sub>3</sub> OC <sub>2</sub> H <sub>4</sub>        | CH <sub>3</sub> OC <sub>2</sub> H <sub>4</sub>        | CH <sub>3</sub>               | 2-CO <sub>2</sub> CH(CH <sub>3</sub> ) <sub>2</sub>                               |
| 15   | C-CN | CH <sub>3</sub> OC <sub>2</sub> H <sub>4</sub>        | CH <sub>3</sub> OC <sub>2</sub> H <sub>4</sub>        | CH <sub>3</sub>               | 2-CO <sub>2</sub> CH <sub>2</sub> CH(CH <sub>3</sub> ) <sub>2</sub>               |
| 16   | C-CN | CH <sub>3</sub> OC <sub>2</sub> H <sub>4</sub>        | CH <sub>3</sub> OC <sub>2</sub> H <sub>4</sub>        | CH <sub>3</sub>               | 2-CO <sub>2</sub> C <sub>2</sub> H <sub>4</sub> CH(CH <sub>3</sub> ) <sub>2</sub> |
| 17   | C-CN | CH <sub>3</sub> OC <sub>2</sub> H <sub>4</sub>        | CH <sub>3</sub> OC <sub>2</sub> H <sub>4</sub>        | CH <sub>3</sub>               | 2-CN                                                                              |
| 18   | C-CN | n-C <sub>4</sub> H <sub>9</sub>                       | n-C <sub>4</sub> H <sub>9</sub>                       | CH <sub>3</sub>               | 2-CN                                                                              |
| 19   | N    | n-C <sub>4</sub> H <sub>9</sub>                       | n-C <sub>4</sub> H <sub>9</sub>                       | CH <sub>3</sub>               | 2-CF <sub>3</sub>                                                                 |
| 20   | N    | n-C <sub>4</sub> H <sub>9</sub>                       | n-C <sub>4</sub> H <sub>9</sub>                       | CH <sub>3</sub>               | 4-NO <sub>2</sub>                                                                 |
| 21   | N    | n-C <sub>4</sub> H <sub>9</sub>                       | n-C <sub>4</sub> H <sub>9</sub>                       | CH <sub>3</sub>               | 2-CN                                                                              |
| 22   | N    | CH <sub>3</sub> OCH <sub>2</sub> (CH <sub>3</sub> )CH | CH <sub>3</sub> OCH <sub>2</sub> (CH <sub>3</sub> )CH | CH <sub>3</sub>               | 2-CF <sub>3</sub>                                                                 |
| 23   | N    | CH <sub>3</sub> OC <sub>2</sub> H <sub>4</sub>        | CH <sub>3</sub> OC <sub>2</sub> H <sub>4</sub>        | CH <sub>3</sub>               | 2-CF <sub>3</sub>                                                                 |

The use of dye mixtures in the dye-donor of the invention permits a wide selection of hue and color that enables a closer hue match to a variety of printing inks and also permits easy transfer of images one or more times to a receiver if desired. The use of dyes also allows easy modification of image density to any desired level. The dyes of the dye-donor element of the invention may be used at a coverage of from about 0.05 to about 1 g/m<sup>2</sup>.

The dyes in the dye-donor of the invention are dispersed in a polymeric binder such as a cellulose derivative, e.g., cellulose acetate hydrogen phthalate, ethyl cellulose, cellulose acetate, cellulose acetate propionate, cellulose acetate butyrate, cellulose triacetate or any of the materials described in U.S. Pat. No. 4,700,207; a polycarbonate; polyvinyl acetate; poly(styrene-co-acrylonitrile); a poly(sulfone) or a poly(phenylene oxide). The binder may be used at a coverage of from about 0.1 to about 5 g/m<sup>2</sup>.

The dye layer of the dye-donor element may be coated on the support or printed thereon by a printing technique such as a gravure process.

Any material can be used as the support for the dye-donor element of the invention provided it is dimensionally stable and can withstand the heat of the laser or thermal head. Such materials include polyesters such as poly(ethylene terephthalate); polyamides; polycarbonates; cellulose esters such as cellulose acetate; fluorine polymers such as polyvinylidene fluoride or poly(tetrafluoroethylene-cohexafluoropropylene); polyethers such as polyoxymethylene; polyacetals; polyolefins such as polystyrene, polyethylene, polypropylene or methylpentene polymers; and polyimides such as polyimide-amides and polyether-imides. The support generally has a thickness of from about 5 to about 200  $\mu$ m. It

may also be coated with a subbing layer, if desired, such as those materials described in U.S. Pat. Nos. 4,695,288 or 4,737,486.

The reverse side of the dye-donor element may be coated with a slipping layer to prevent the printing head from sticking to the dye-donor element. Such a slipping layer would comprise either a solid or liquid lubricating material or mixtures thereof, with or without a polymeric binder or a surface active agent. Preferred lubricating materials include oils or semi-crystalline organic solids that melt below 100° C. such as poly(vinyl stearate), beeswax, perfluorinated alkyl ester polyethers, poly(capro-lactone), silicone oil, poly(tetrafluoroethylene), carbowax, poly(ethylene glycols), or any of those materials disclosed in U.S. Pat. Nos. 4,717,711; 4,717,712; 4,737,485; and 4,738,950. Suitable polymeric binders for the slipping layer include poly(vinyl alcohol-co-butyral), poly(vinyl alcohol-co-acetal), poly(styrene), poly(vinyl acetate), cellulose acetate butyrate, cellulose acetate propionate, cellulose acetate or ethyl cellulose.

The amount of the lubricating material to be used in the slipping layer depends largely on the type of lubricating material, but is generally in the range of about 0.001 to about 2 g/m<sup>2</sup>. If a polymeric binder is employed, the lubricating material is present in the range of 0.1 to 50 weight %, preferably 0.5 to 40, of the polymeric binder employed.

The dye-receiving element that is used with the dye-donor element of the invention usually comprises a support having thereon a dye image-receiving layer. The support may be a transparent film such as a poly(ether sulfone), a polyimide, a cellulose ester such as cellulose acetate, a poly(vinyl alcohol-co-acetal) or a poly-

(ethylene terephthalate). The support for the dye-receiving element may also be reflective such as baryta-coated paper, polyethylene-coated paper, an ivory paper, a condenser paper or a synthetic paper such as duPont Tyvek®. Pigmented supports such as white polyester (transparent polyester with white pigment incorporated therein) may also be used.

The dye image-receiving layer may comprise, for example, a polycarbonate, a polyurethane, a polyester, polyvinyl chloride, poly(styrene-coacrylonitrile), poly(caprolactone), a poly(vinyl acetal) such as poly(vinyl alcohol-co-butyl), poly(vinyl alcohol-co-benzal), poly(vinyl alcohol-coacetal) or mixtures thereof. The dye image-receiving layer may be present in any amount which is effective for the intended purpose. In general, good results have been obtained at a concentration of from about 1 to about 5 g/m<sup>2</sup>.

As noted above, the dye-donor elements of the invention are used to form a dye transfer image. Such a process comprises imagewise-heating a dye-donor element as described above and transferring a dye image to a dye-receiving element to form the dye transfer image.

The dye-donor element of the invention may be used in sheet form or in a continuous roll or ribbon. If a continuous roll or ribbon is employed, it may have only the yellow dyes thereon as described above or may have alternating areas of other different dyes or combinations, such as sublimable cyan and/or magenta and/or black or other dyes. Such dyes are disclosed in U.S. Pat. No. 4,541,830, the disclosure of which is hereby incorporated by reference. Thus, one-, two-, three- or four-color elements (or higher numbers also) are included within the scope of the invention.

Thermal printing heads which can be used to transfer dye from the dye-donor elements of the invention are available commercially. There can be employed, for example, a Fujitsu Thermal Head (FTP-040 MCS001), a TDK Thermal Head F415 HH7-1089 or a Rohm Thermal Head KE 2008-F3.

A laser may also be used to transfer dye from the dye-donor elements of the invention. When a laser is used, it is preferred to use a diode laser since it offers substantial advantages in terms of its small size, low cost, stability, reliability, ruggedness, and ease of modulation. In practice, before any laser can be used to heat a dye-donor element, the element must contain an infrared-absorbing material, such as carbon black, cyanine infrared absorbing dyes as described in DeBoer application Ser. No. 463,095, filed Jan. 10, 1990, or other materials as described in the following U.S. application Ser. Nos.: 366,970, 67,062, 366,967, 366,968, 366,969, 367,064, 367,061, 69,494, 366,952, 369,493, 369,492, and 369,491, the disclosures of which are hereby incorporated by reference. The laser radiation is then absorbed into the dye layer and converted to heat by a molecular process known as internal conversion. Thus, the construction of a useful dye layer will depend not only on the hue, transferability and intensity of the image dyes, but also on the ability of the dye layer to absorb the radiation and convert it to heat.

Lasers which can be used to transfer dye from dye-donors employed in the invention are available commercially. There can be employed, for example, Laser Model SDL-2420-H2 from Spectra Diode Labs, or Laser Model SLD 304 V/W from Sony Corp.

A thermal printer which uses the laser described above to form an image on a thermal print medium is described and claimed in copending U.S. application

serial No. 451,656 of Baek and DeBoer, filed Dec. 18, 1989, the disclosure of which is hereby incorporated by reference.

Spacer beads may be employed in a separate layer over the dye layer of the dye-donor in the above-described laser process in order to separate the dye-donor from the dye-receiver during dye transfer, thereby increasing the uniformity and density of the transferred image. That invention is more fully described in U.S. Pat. No. 4,772,582, the disclosure of which is hereby incorporated by reference. Alternatively, the spacer beads may be employed in the receiving layer of the dye-receiver as described in U.S. Pat. No. 4,876,235, the disclosure of which is hereby incorporated by reference. The spacer beads may be coated with a polymeric binder if desired.

The use of an intermediate receiver with subsequent retransfer to a second receiving element may also be employed in the invention. A multitude of different substrates can be used to prepare the color proof (the second receiver) which is preferably the same substrate used for the printing press run. Thus, this one intermediate receiver can be optimized for efficient dye uptake without dye-smearing or crystallization.

Examples of substrates which may be used for the second receiving element (color proof) include the following: Flo Kote Cove® (S. D. Warren Co.), Champion Textweb® (Champion Paper Co.), Quintessence Gloss® (Potlatch Inc.), Vintage Gloss® (Potlatch Inc.), Khrome Kote® (Champion Paper Co.), Ad-Proof Paper® (Appleton Papers, Inc.), Consolith Gloss® (Consolidated Papers Co.) and Mountie Matte® (Potlatch Inc.).

As noted above, after the dye image is obtained on a first dye-receiving element, it is retransferred to a second dye image-receiving element. This can be accomplished, for example, by passing the two receivers between a pair of heated rollers. Other methods of retransferring the dye image could also be used such as using a heated platen, use of pressure and heat, external heating, etc.

Also as noted above, in making a color proof, a set of electrical signals is generated which is representative of the shape and color of an original image. This can be done, for example, by scanning an original image, filtering the image to separate it into the desired additive primary colors-red, blue and green, and then converting the light energy into electrical energy. The electrical signals are then modified by computer to form the color separation data which is used to form a halftone color proof. Instead of scanning an original object to obtain the electrical signals, the signals may also be generated by computer. This process is described more fully in Graphic Arts Manual, Janet Field ed., Arno Press, New York 1980 (p. 358ff), the disclosure of which is hereby incorporated by reference.

A thermal dye transfer assemblage of the invention comprises

a) a dye-donor element as described above, and  
b) a dye-receiving element as described above, the dye-receiving element being in a superposed relationship with the dye-donor element so that the dye layer of the donor element is in contact with the dye image-receiving layer of the receiving element.

The above assemblage comprising these two elements may be preassembled as an integral unit when a monochrome image is to be obtained. This may be done by temporarily adhering the two elements together at their

margins. After transfer, the dye-receiving element is then peeled apart to reveal the dye transfer image.

When a three-color image is to be obtained, the above assemblage is formed three times using different dye-donor elements. After the first dye is transferred, the elements are peeled apart. A second dye-donor element (or another area of the donor element with a different dye area) is then brought in register with the dye-receiving element and the process repeated. The third color is obtained in the same manner.

The following examples are provided to illustrate the invention.

### EXAMPLE 1

Individual yellow dye-donor elements were prepared by coating on a 100  $\mu\text{m}$  poly(ethylene terephthalate) support:

- 1) a subbing layer of poly(acrylonitrile-covinylidene chloride-co-acrylic acid) (0.054 g/m<sup>2</sup>) (14:79:7 wt. ratio); and
- 2) a dye layer containing a mixture of the yellow dyes identified below and illustrated above, (total coverage 0.27 g/m<sup>2</sup>) and the cyanine infrared absorbing dye illustrated below (0.054 g/m<sup>2</sup>) in a cellulose acetate propionate binder (2.5% acetyl, 45% propionyl) (0.27 g/m<sup>2</sup>) coated from dichloromethane.

Comparison dye-donors using the individual yellow dyes of the mixture and a control dye-donor with a single yellow dye identified below, each at 0.27 g/m<sup>2</sup>, were also prepared.

optical fiber (100 microns core diameter) was imaged onto the plane of the dye-donor with a 0.33 magnification lens assembly mounted on a translation stage giving a nominal spot size of 33 microns and a measured power output at the focal plane of 115 milliwatts.

The drum, 312 mm in circumference, was rotated at 500 rpm and the imaging electronics were activated. The translation stage was incrementally advanced across the dye-donor by means of a lead screw turned by a microstepping motor, to give a center-to-center line distance of 14 microns (714 lines per centimeter, or 1800 lines per inch). For a continuous tone stepped image, the current supplied to the laser was modulated from full power to 16% power in 4% increments.

After the laser had scanned approximately 12 mm, the laser exposing device was stopped and the intermediate receiver was separated from the dye donor. The intermediate receiver containing the stepped dye image was laminated to Ad-Proof Paper® (Appleton Papers, Inc.) 60 pound stock paper by passage through a pair of rubber rollers heated to 120°C. The polyethylene terephthalate support was then peeled away leaving the dye image and polyvinyl alcohol-co-butylal firmly adhered to the paper. The paper stock was chosen to represent the substrate used for a printed ink image obtained from a printing press.

The Status T density of each of the stepped images was read using an X-Rite® 418 Densitometer to find the single step image within 0.05 density unit of the 30 SWOP Color Reference. For the yellow standard, this

Cyanine Infrared Absorbing Dye



An intermediate dye-receiving element was prepared by coating on an unsubbed 100  $\mu\text{m}$  thick poly(ethylene terephthalate) support a layer of crosslinked poly(styrene-co-divinylbenzene) beads (14 micron average diameter) (0.11 g/m<sup>2</sup>), triethanolamine (0.09 g/m<sup>2</sup>) and DC-510® Silicone Fluid (Dow Corning Company) (0.01 g/m<sup>2</sup>) in a Butvar® 76 binder, a poly(vinyl alcohol-co-butylal), (Monsanto Company) (4.0 g/m<sup>2</sup>) from 1,1,2-trichloroethane or dichloromethane.

Single color images were printed as described below from dye-donors onto the above receiver using a laser imaging device as described in U.S. Pat. No. 4,876,235. The laser imaging device consisted of a single diode laser connected to a lens assembly mounted on a translation stage and focused onto the dye-donor layer.

The dye-receiving element was secured to the drum 60 of the diode laser imaging device with the receiving layer facing out. The dye-donor element was secured in face-to-face contact with the receiving element.

The diode laser used was a Spectra Diode Labs No. 65 SDL-2430-H2, having an integral, attached optical fiber for the output of the laser beam, with a wavelength of 816 nm and a nominal power output of 250 milliwatts at the end of the optical fiber. The cleaved face of the

density was 1.0.

The a\* and b\* values of the selected step image of transferred dye or dye-mixture was compared to that of the SWOP Color Reference by reading on an X-Rite® 918 Colorimeter set for D50 illuminant and a 10 degree observer. The L\* reading was checked to see that it did not differ appreciably from the reference. The a\* and b\* readings were recorded and the distance from the SWOP Color Reference calculated as the square root of the sum of differences squared for a\* and b\*:

$$\text{i.e. } \sqrt{(a^*_{\text{e}} - a^*_{\text{s}})^2 + (b^*_{\text{e}} - b^*_{\text{s}})^2}$$

e = experiment (transferred dye)

s = SWOP Color Reference

The following results were obtained:

TABLE 1

| Dye(s)<br>(Wt. Ratio) | a*  | b*   | Distance From<br>Reference |
|-----------------------|-----|------|----------------------------|
| SWOP                  | 2.3 | 84.8 | —                          |

TABLE 1-continued

| Dye(s)<br>(Wt. Ratio) | a*   | b*   | Distance From<br>Reference | 5 |
|-----------------------|------|------|----------------------------|---|
| A                     | -6.0 | 74.6 | 13                         |   |
| A/1 (60:40)           | 5.6  | 84.4 | 3                          |   |
| 1                     | 10.5 | 73.7 | 14                         |   |
| Control*              | -0.9 | 98.6 | 14                         |   |

\*U.S. Pat. No. 4,923,846, Table C-2 (Example C-2), Foron Brilliant Yellow S-6GL 10 having the following structure:



The above results indicate that by using a mixture of 20 the dyes according to the invention in an appropriate ratio, a hue closely corresponding to that of the yellow SWOP Color Reference was obtained, in comparison to the control or individual yellow dye images which were 25 much further away from the SWOP Color Reference.

The invention has been described in detail with particular reference to preferred embodiments thereof, but it will be understood that variations and modifications 30 can be effected within the spirit and scope of the invention.

What is claimed is:

1. A yellow dye-donor element for thermal dye transfer comprising a support having thereon a dye layer comprising a mixture of yellow dyes dispersed in a polymeric binder, at least one of said yellow dyes having the formula:



wherein:

R<sup>1</sup> represents hydrogen or halogen;

each R<sup>2</sup> independently represents hydroxy, alkoxy, aryloxy, acyloxy, aminocarbonyl, carbamoyloxy, halogen, aryl, hetaryl, cyano, acylamido, alkoxy-carbonyl, alkylthio, arylthio, alkylsulfonyl, arylsulfonyl, alkylsulfonamido or arylsulfonamido; or any two adjacent R<sup>2</sup>'s together represent the atoms necessary to complete a 5- or 6-membered fused saturated or aromatic ring;

Y represents H or OH; and

n is an integer from 0 to 4;

and at least one of the other of the dyes having the formula:



wherein:

R<sup>3</sup> and R<sup>4</sup> each independently represents a substituted or unsubstituted alkyl group of from 1 to about 6 carbon atoms, a cycloalkyl group of from about 5 to about 7 carbon atoms; a substituted or unsubstituted allyl group; an aryl group of from about 6 to about 10 carbon atoms; a hetaryl group of from 5 to 10 atoms; acyl; arylsulfonyl; aminocarbonyl; aminosulfonyl; fluorosulfonyl; halogen; nitro; alkylthio; or arylthio;

R<sup>5</sup> represents H, a substituted or unsubstituted alkyl, allyl, aryl or hetaryl group as described above for R<sup>3</sup>; halogen; carbamoyl; cyano; or alkoxy carbonyl; each R<sup>6</sup> independently represents substituted or unsubstituted alkyl, aryl, allyl or hetaryl groups such as those listed above for R<sup>3</sup>; hydroxy, alkoxy, aryloxy, acyloxy, aminocarbonyl, aminosulfonyl, carbamoyloxy, halogen, aryl, cyano, nitro, trifluoromethyl, fluorosulfonyl, acylamido, alkoxy carbonyl, alkylthio, arylthio, alkylsulfonyl, arylsulfonyl, alkylsulfonamido or arylsulfonamido; or two adjacent R<sup>6</sup>'s together represent the atoms necessary to complete a 5- or 6-membered fused saturated or aromatic ring;

X represents CR<sup>7</sup> or N;

R<sup>7</sup> represents the same groups as R<sup>5</sup>; and

m is an integer from 0 to 5.

2. The element of claim 1 wherein R<sup>1</sup> is hydrogen.

3. The element of claim 1 wherein R<sup>2</sup> is hydrogen.

4. The element of claim 1 wherein Y is hydrogen.

5. The element of claim 1 wherein X is C—CN.

6. The element of claim 1 wherein R<sup>3</sup> is CH<sub>3</sub>OC<sub>2</sub>H<sub>4</sub> or n—C<sub>4</sub>H<sub>9</sub>.

7. The element of claim 1 wherein R<sup>4</sup> is CH<sub>3</sub>OC<sub>2</sub>H<sub>4</sub> or n—C<sub>4</sub>H<sub>9</sub>.

8. The element of claim 1 wherein R<sup>5</sup> is CH<sub>3</sub> or C<sub>6</sub>H<sub>5</sub>.

9. The element of claim 1 wherein R<sup>6</sup> is CN, OCH<sub>3</sub> or CO<sub>2</sub>C<sub>2</sub>H<sub>5</sub>.

10. The element of claim 1 wherein said dye-donor element contains an infrared-absorbing dye in said dye layer.

11. The element of claim 1 wherein R<sup>1</sup>, R<sup>2</sup> and Y are each hydrogen, n is 1, R<sup>3</sup> and R<sup>4</sup> are each CH<sub>3</sub>OC<sub>2</sub>H<sub>4</sub>, R<sup>5</sup> is CH<sub>3</sub>, R<sup>6</sup> is 2,5—(OCH<sub>3</sub>)<sub>2</sub>, X is C—CN and m is 2.

12. In a process of forming a dye transfer image comprising imagewise-heating a yellow dye-donor element comprising a support having thereon a dye layer comprising a mixture of yellow dyes dispersed in a polymeric binder and transferring a yellow dye image to a dye-receiving element to form said yellow dye transfer image, the improvement wherein at least one of said yellow dyes has the formula:



wherein:

R¹ represents hydrogen or halogen;  
each R² independently represents hydroxy, alkoxy, aryloxy, acyloxy, aminocarbonyl, carbamoyloxy, halogen, aryl, hetaryl, cyano, acylamido, alkoxy-carbonyl, alkylthio, arylthio, alkylsulfonyl, arylsulfonyl, alkylsulfonamido or arylsulfonamido; or any two adjacent R²'s together represent the atoms necessary to complete a 5- or 6-membered fused saturated or aromatic ring;

Y represents H or OH; and  
n is an integer from 0 to 4;  
or any two adjacent R¹'s together represent the atoms necessary to form a 5- or 6-membered fused ring;

n represents an integer from 0-4;

and at least one of the other of the dyes having the formula:



wherein:

R³ and R⁴ each independently represents a substituted or unsubstituted alkyl group of from 1 to about 6 carbon atoms, a cycloalkyl group of from about 5 to about 7 carbon atoms; a substituted or unsubstituted allyl group; an aryl group of from about 6 to about 10 carbon atoms; a hetaryl group of from 5 to 10 atoms; acyl; arylsulfonyl; aminocarbonyl; aminosulfonyl; fluorosulfonyl; halogen; nitro; alkylthio; or arylthio;

R⁵ represents H, a substituted or unsubstituted alkyl, allyl, aryl or hetaryl group as described above for R³; halogen; carbamoyl; cyano; or alkoxy carbonyl; each R⁶ independently represents substituted or unsubstituted alkyl, aryl, allyl or hetaryl groups such as those listed above for R³; hydroxy, alkoxy, aryloxy, acyloxy, aminocarbonyl, aminosulfonyl, carbamoyloxy, halogen, aryl, cyano, nitro, trifluoromethyl, fluorosulfonyl, acylamido, alkoxy carbonyl, alkylthio, arylthio, alkylsulfonyl, arylsulfonyl, alkylsulfonamido or arylsulfonamido; or two adjacent R⁶'s together represent the atoms necessary to complete a 5- or 6-membered fused saturated or aromatic ring;

X represents CR⁷ or N;

R⁷ represents the same groups as R⁵; and  
m is an integer from 0 to 5.

13. The process of claim 12 wherein R¹, R² and Y are each hydrogen, n is 1, R³ and R⁴ are each CH<sub>3</sub>OC<sub>2</sub>H<sub>4</sub>, R⁵ is CH<sub>3</sub>, R⁶ is 2,5-(OCH<sub>3</sub>)<sub>2</sub>, X is C—CN and m is 2.

14. In a thermal dye transfer assemblage comprising:  
a) a yellow dye-donor element comprising a support having thereon a dye layer comprising a mixture of yellow dyes dispersed in a polymeric binder,  
b) a dye-receiving element comprising a support having thereon a dye image-receiving layer, said dye-receiving element being in a superposed relationship with said yellow dye-donor element so that said dye layer is in contact with said dye image-receiving layer, the improvement wherein at least one of said yellow dyes has the formula:



wherein:

R¹ represents hydrogen or halogen;  
each R² independently represents hydroxy, alkoxy, aryloxy, acyloxy, aminocarbonyl, carbamoyloxy, halogen, aryl, hetaryl, cyano, acylamido, alkoxy-carbonyl, alkylthio, arylthio, alkylsulfonyl, arylsulfonyl, alkylsulfonamido or arylsulfonamido; or any two adjacent R²'s together represent the atoms necessary to complete a 5- or 6-membered fused saturated or aromatic ring;

Y represents H or OH; and  
n is an integer from 0 to 4;  
or any two adjacent R¹'s together represent the atoms necessary to form a 5- or 6-membered fused ring;

n represents an integer from 0-4;

and at least one of the other of the dyes having the formula:



wherein:

R³ and R⁴ each independently represents a substituted or unsubstituted alkyl group of from 1 to about 6 carbon atoms, a cycloalkyl group of from about 5 to about 7 carbon atoms; a substituted or unsubstituted allyl group; an aryl group of from about 6 to about 10 carbon atoms; a hetaryl group of from 5 to 10 atoms; acyl; arylsulfonyl; aminocarbonyl; aminosulfonyl; fluorosulfonyl; halogen; nitro; alkylthio; or arylthio;

R⁵ represents H, a substituted or unsubstituted alkyl, allyl, aryl or hetaryl group as described above for R³; halogen; carbamoyl; cyano; or alkoxy carbonyl;

each R<sup>6</sup> independently represents substituted or unsubstituted alkyl, aryl, allyl or hetaryl groups such as those listed above for R<sup>3</sup>; hydroxy, alkoxy, aryloxy, acyloxy, aminocarbonyl, aminosulfonyl, carbamoyloxy, halogen, aryl, cyano, nitro, trifluoromethyl, fluorosulfonyl, acylamido, alkoxy carbonyl, alkylthio, arylthio, alkylsulfonyl, arylsulfonyl, alkylsulfonamido or arylsulfonamido; or two adjacent R<sup>6</sup>'s together represent the atoms neces-

10

sary to complete a 5- or 6-membered fused saturated or aromatic ring;

X represents CR<sup>7</sup> or N;

R<sup>7</sup> represents the same groups as R<sup>5</sup>; and

m is an integer from 0 to 5.

15. The assemblage of claim 14 wherein R<sup>1</sup>, R<sup>2</sup> and Y are each hydrogen, n is 1, R<sup>3</sup> and R<sup>4</sup> are each CH<sub>3</sub>OC<sub>2</sub>H<sub>4</sub>, R<sup>5</sup> is CH<sub>3</sub>, R<sup>6</sup> is 2,5—(OCH<sub>3</sub>)<sub>2</sub>, X is C—CN and m is 2.

\* \* \* \* \*

15

20

25

30

35

40

45

50

55

60

65